

# UNITED STATES PATENT OFFICE.

WILLIAM D. COOLIDGE, OF SCHENECTADY, NEW YORK, ASSIGNOR TO GENERAL ELECTRIC COMPANY, A CORPORATION OF NEW YORK.

## METAL FILAMENT.

1,026,383.

Specification of Letters Patent. Patented May 14, 1912.

No Drawing.

Application filed May 9, 1908. Serial No. 316,006.

*To all whom it may concern:*

Be it known that I, WILLIAM DAVID COOLIDGE, a citizen of the United States, residing at Schenectady, in the county of Schenectady and State of New York, have invented certain new and useful Improvements in Metal Filaments, of which the following is a specification.

This invention relates to the production of filaments suitable for use in incandescent electric lamps.

Various refractory metals, such as tungsten and molybdenum, have heretofore been proposed for use in incandescent lamps, but difficulty has been experienced in shaping the metal into filaments of suitable length and cross-section. These refractory metals are usually obtained as fine powders, and some special process must be resorted to in producing lamp filaments therefrom.

According to this invention an amalgam is used to bind the particles of refractory metal together and to make a semi-plastic mass which may be squirted or otherwise shaped into wires which on subsequent treatment may be converted into lamp filaments containing nothing but the refractory metal.

Although my process is applicable to the treatment of various refractory metals and materials such as tungsten, molybdenum, boron, zirconium, titanium, etc., I will explain the process as applied to the treatment of tungsten, and it is to be understood that the process is also applicable to other refractory metals, elements and compounds.

An amalgam is made by melting together cadmium and mercury in about equal parts by weight. This amalgam fuses at a low temperature and can readily be made very uniform in composition. To this amalgam is added the refractory metal, such as tungsten, in a finely divided condition. The tungsten is thoroughly rubbed into the amalgam while the latter is at such a temperature as to be plastic, in any suitable way, as with a pestle in an ordinary chemist's mortar. I do not think that the tungsten unites chemically with the cadmium amalgam or that a tungsten alloy of any kind is formed. I believe that the mixture is merely a mechanical one in which the cadmium amalgam serves as a binding ma-

terial to hold together the particles of finely divided tungsten. I consider it advisable to add tungsten until the mixture contains about 55 per cent. by weight of tungsten. The mixture of tungsten and cadmium amalgam is then squirted warm through a die and comes out as a silver white ductile wire. It can be squirted in sizes of small diameter, or it can be squirted in sizes of about 1/100 of an inch and then drawn down through a suitable draw plate to smaller sizes suitable for use in lamps operative on commercial voltages.

The next step in my process consists in the removal of the mercury and cadmium from the wire to leave a filament of pure refractory metal. This may be done by heating it in a vacuum, or in a hydrogen atmosphere. I find it desirable to heat the wires slowly to prevent a sudden distillation of the cadmium and mercury from the wire. When thus gradually heated, a part of the mercury seems to pass off first, and is followed by a mixture of cadmium and mercury, until the tungsten or other refractory metal has been completely freed from the other metallic components of the original squirted wire.

I consider it desirable to heat the wire during the distillation just described by current passed through the wire, and when the distillation is substantially complete I increase the current to sinter the particles of tungsten together and produce a strong, compact filament.

In certain of the claims appended hereto I have used the word "metal", but I desire it to be understood that this term is used in the popular sense of either a metallic element, an alloy, or a metallic mixture.

What I claim as new and desire to secure by Letters Patent of the United States, is,

1. A ductile wire composed of an amalgam impregnated with finely divided refractory metal.
2. A conducting wire consisting of finely divided refractory metal the particles of which are cemented together with an amalgam.
3. The composition of matter consisting of a mixture of cadmium amalgam and a powdered refractory metal.
4. The composition of matter consisting

of an amalgam impregnated with tungsten.

5. The composition of matter consisting of cadmium amalgam and finely divided tungsten.

6. A wire composed of powdered material mixed with and held in place by a cadmium mercury alloy.

In witness whereof, I have hereunto set my hand this 8th day of May, 1906.

WILLIAM D. COOLIDGE.

Witnesses:

BENJAMIN B. HULL,  
HELEN ORFORD.